# EUROPEAN PATENT APPLICATION

(11) **EP 0 897 764 A1**
(43) Date of publication of application: **24.02.1999**
(21) Application number: 98200551.4
(22) Date of filing: 20.02.1998
(51) Int. Cl.: B21C 1/22, C22F 1/08

(54) **Method of manufacturing a (copper) tube which is insensitive to stress corrosion**

(71) Applicant: HME Nederland B.V., 5151 RP Drunen (NL)
(72) Inventor: The designation of the inventor has not yet been filed
(74) Representative: Smulders, Theodorus A.H.J., Ir.

(57) **Abstract**

A method of manufacturing a copper tube, which method comprises at least the following method step:
-a. the copper tube is sunk;
   wherein the method further comprises at least the following method step:
-b. the copper tube is plastically stretched;
   which method step b. is carried out after method step a.
The half-hard or hard tube thus manufactured has a very low value for the residual hoop stress. Consequently, the tube is very insensitive to stress corrosion.

## Description

The invention relates to a method of manufacturing a copper tube, which method comprises at least the following method step:
-a. the copper tube is sunk.
It is known that hard and half-hard drawn copper tubes manufactured according to the above method are sensitive to stress corrosion, depending on the internal stress level and the internal stress distribution. In the known method at least one drawing reduction is often carried out before the sinking reduction (this is drawing without a drawing plug). To obtain a half-hard tube, the tube is annealed at a temperature of e.g. 600°C after carrying out the drawing treatment(s) and before carrying out the sinking.

A study has shown that the tubes manufactured according to the known method have an unfavorable internal stress distribution, as a result of which this tube is sensitive to stress corrosion.

The copper tubes thus manufactured are mostly processed on the spot. The tubes then come into external contact with various building materials and often also with cleaning agents which contain substances that may cause stress corrosion. To make the mortar properly processable, agents are often added to this mortar. The tube insulating material too may contain harmful substances in relation to sensitivity to stress corrosion. Stress corrosion develops if the following conditions are satisfied (see DIN 50900):
a. moist surroundings;
b. sufficient tensile stress (internal and/or external); and
c. presence of specific chemicals.

If one of these three components is not present, stress corrosion does not occur. It is further known that the microstructure of the material too may influence the development of stress corrosion.

The object of the invention is to provide a method of manufacturing a copper tube with such a low tangential tensile stress that it becomes insensitive to stress corrosion.

The invention is therefore characterized in that the method further comprises the following method step:
-b. the copper tube is plastically stretched;
   which method step b. is carried out after method step a.

The invention is based on the insight that during the sinking of the copper tube the tangential stress in the tube can run very high. This internal tangential stress is often expressed in residual hoop stress. An approximation of the tangential stress in the wall of a tube can be calculated from the amount of "springiness" which becomes visible after sawing the tube through in the longitudinal direction. Practically speaking, this means that a tube sample being ca. 30 mm in length is used for this measurement. Both before and after sawing through the diameter is measured at 90° displacement relative to the saw cut. The residual hoop stress can be calculated by means of the following formula:${\text{σ}}_{\text{c}} \text{= E'} \text{t} \left(\frac{\text{1}}{\text{D} \text{0}} \text{-} \frac{\text{1}}{\text{D} \text{1}}\right)$ wherein
- σ_{c}: = Residual hoop stress (N/mm²)
- E': = ${\text{E/(1-v}}^{\text{2}} {\text{) (N/mm}}^{\text{2}} \text{)}$
- E: = Young's modulus (N/mm²)
- v: = Poisson's ratio
- D₀: = Diameter before sawing through (mm)
- D₁: = Diameter after sawing through (mm)
- t: = Wall thickness (mm)

After sinking, the tubes have a residual hoop stress value which, depending on the diameter reduction, can increase during the sinking to a value of 30 to 200 and even more. In the known tube, this causes the above sensitivity to stress corrosion. When, according to the invention, the copper tube is plastically stretched after sinking, it appears that the internal tangential stress is nearly completely reduced to zero. The stretching in method step b. is carried out below the recrystallisation temperature of the tube. The residual hoop stress of the tube then has a value below 30. This results in the tube thus obtained being insensitive to stress corrosion.

In particular, it applies that the copper tube in step a. is at least substantially drawn to a final dimension through sinking. It further applies that, in particular, the copper tube in step b. is extended by 0.05 to 5%.

According to the invention, both hard and half-hard tubes can be manufactured. According to a special variant of the invention, method step a. is preceded by the following method step:
-c. the copper tube is annealed for manufacturing a half-hard copper tube.

Through annealing, the copper tube softens. To bring the tube into the half-hard condition after annealing, the tube is drawn through a die without a plug. In other words, after annealing a sinking reduction is carried out for manufacturing a half-hard tube.

Both to the manufacture of a hard tube and to a half-hard tube it applies that according to the invention method step b. is preferably carried out immediately after method step a.

It should be noted that in the manufacture of a copper tube it is known per se to carry out a stretching treatment. Cold plastic stretching, however, then aims to direct the copper tube. According to the invention, the plastic stretching of the copper tube is carried out after the copper tube has experienced a sinking reduction.

The invention will now be explained in more detail with reference to some practical examples.

The starting product for manufacturing a copper tube consists of:
1) a copper cast bar which is converted into a copper tube by means of extrusion or piercing; or
2) a cast copper tube.

This copper tube is first pilgered depending on its dimension and then subjected to at least one drawing treatment. When carrying out the drawing treatment, the length of the tube is substantially extended. Drawing machines known per se may be used therefor, which will hereinafter not be discussed any further. After the copper tube has experienced at least one and in general a number of such drawing treatments, it is hard. To soften the tube, it is annealed at a temperature of 500-700°C. More in particular, the copper tube is annealed at a temperature of about 600°C. The tube is then soft. Subsequently, the soft tube is subjected to a drawing treatment in which no drawing plug is used. Such a treatment is also called a sinking reduction. In other words, the copper tube is sunk. During the sinking reduction the copper tube is at least substantially drawn to a final dimension. After the sinking reduction the copper tube has the half-hard quality.
In Figure 1 curve I indicates how the residual hoop stress of the copper tube increases depending on the diameter reduction of the copper tube during the sinking. Apparently, it can increase from a value zero to 140 if a soft tube is sunk.

An estimation of the residual hoop stress in a tube can be obtained as follows.

The diameter of a section of the tube being about 30 mm in length is measured. Subsequently, perpendicular to the diameter measured, a slot is provided in the longitudinal direction of the tube wall. Then the diameter of the tube is measured again in the original place. The residual hoop stress is determined as follows:${\text{σ}}_{\text{c}} \text{= E'} \text{t} \left(\frac{\text{1}}{\text{D} \text{0}} \text{-} \frac{\text{1}}{\text{D} \text{1}}\right)$ wherein
- σ_{c}: = Residual hoop stress (N/mm²)
- E': = ${\text{E/(1-v}}^{\text{2}} {\text{) (N/mm}}^{\text{2}} \text{)}$
- E: = Young's modulus (N/mm²)
- v: = Poisson's ratio
- D₀: = Diameter before sawing through (mm)
- D₁: = Diameter after sawing through (mm)
- t: = Wall thickness (mm)
To carry out the calculation, it is assumed that E = 112 GPa and v = 0.343.

The residual hoop stress is plotted on the vertical axis of Figure 1. Plotted in percentages on the horizontal axis is the diameter reduction during the sinking of the tube.

According to the invention the copper tube is plastically stretched after sinking. This stretching is carried out at a temperature below the recrystallisation temperature of the tube. It appears that after stretching the residual hoop stress falls to a value below 30. As a result, the tube is very insensitive to stress corrosion. In particular, it applies that the copper tube in step a. is at least substantially drawn to a final dimension through sinking. This is also apparent from the fact that the copper tube in step b. is extended by 0.05-5%. Method step a. is then the last drawing step. In particular, it applies that the copper tube in step b. is extended between 0.2 and 3%.

In particular, it further applies that in step b. the copper tube experiences a diameter reduction below 0.5%. Preferably, it applies that the copper tube in method step b. experiences a diameter reduction below 0.2%.

According to a further elaboration of the invention it applies that the copper tube in method step a. experiences a diameter reduction of 2-20%. In particular, it also applies that the copper tube in step a. experiences a diameter reduction of 1-4 mm and has a diameter of 6-42 mm after carrying out this method step. This is then also at least substantially the diameter of the final product.

In particular, it applies that method step b. is carried out immediately after method step a. In this example drawing treatments preceding method step c. are cold drawing treatments, i.e. drawing treatments below the recrystallisation temperature of the tube.

The final product thus obtained has a residual hoop stress below 30 and may even approach zero. After the sinking reduction was carried out and before the tube was stretched the residual hoop stress had a value above 30 and in particular even a value that may range from 30 to 200. The tremendous advantage of the invention is therefore that by means of stretching the negative effects of sinking are completely reduced and even more than that.

The above-described method may also be carried out to manufacture tubes of any desired hardness with the exception of soft. The difference is that the above annealing treatment, i.e. method step c., is omitted or not. This means that before the sinking reduction the copper tube is subjected to at least one drawing treatment.

In Figure 1 curve II indicates the extent to which the residual hoop stress of a hard tube increases when it is subjected to a sinking reduction. It appears that the residual hoop stress in a hard tube is even higher than in half-hard tube. It also applies to the hard tube that this residual hoop stress is reduced again to a value below 30 b carrying out a stretching treatment following the sinking reduction, as discussed above in relation to the half-hard tube.

It also applies to the carrying out of the sinking reduction after the annealing treatment and before the stretching treatment that devices known per se may be used. These devices will therefore not be discussed any further. The tube may be stretched, e.g., with a draw bench known per se.

An example of a method not carried out according to the invention and of a method carried out according to the invention is given below.

### Example 1 (not according to the invention)

The starting product is a copper cast bar which is converted into a copper tube by means of extrusion. This copper tube has a length of 150 m, an outside diameter of 31 mm, and an inside diameter of 27.5 mm. This tube is subjected to a first cold drawing treatment. After carrying out the drawing treatment, the tube has a length of ca. 238.8 m, an outside diameter of 28 mm, and an inside diameter of 25.6 mm. Subsequently, the tube is subjected to a second drawing treatment. After carrying out the second drawing treatment, the tube has a length of 320 m, an outside diameter of 25 mm, and an inside diameter of 23 mm. The tube thus obtained is gently annealed at a temperature of 600°C. Subsequently, by means of a sinking reduction the tube is at least substantially drawn to the final dimension. When carrying out the sinking reduction, which is a drawing treatment without using a drawing plug, the tube obtains its half-hard quality. The final tube dimension thus obtained is as follows: the tube has a length of 365.6 m, an outside diameter of 22 mm, and an inside diameter of 20 mm. The value measured for the residual hoop stress is 120. Since the residual hoop stress has a high value, it appears that the copper tube is very sensitive to stress corrosion.

### Example 2 according to the invention

The starting product is a copper casting bar which is converted into a copper tube by means of extrusion. This copper tube has a length of 150 m, an outside diameter of 31 mm, and an inside diameter of 27.5 mm. This tube is subjected to a first drawing treatment. After carrying out the drawing treatment, the tube has a length of 238.8 m, an outside diameter of 28 mm, and an inside diameter of 25.6 mm. Subsequently, the tube is subjected to a second drawing treatment. After carrying out the second drawing treatment, the tube has a length of 320 m, an outside diameter of 25 mm, and an inside diameter of 23 mm. The tube thus obtained is gently annealed at a temperature of 600°C. Subsequently, by means of a sinking reduction the tube is at least substantially drawn to the final dimension. The sinking reduction is therefore the last drawing treatment. When carrying out the sinking reduction, which is a drawing treatment without using a drawing plug, the tube is half-hard. The tube dimension thus obtained is as follows: the tube has a length of 356.6 m, an outside diameter of 22.05 mm, and an inside diameter of 20.05 mm. The value measured for the residual hoop stress is 120. Subsequently, the tube is subjected to a stretching treatment. The tube then has a temperature below the recrystallisation temperature of the tube. During stretching, the tube is extended by 0.5%. After extension the outside diameter is 22 mm, and the inside diameter 20 mm. It appears that the residual hoop stress now has a value of 23.

The invention is by no means limited to the above-described embodiments. To obtain a hard tube, the annealing treatment can be left out in Example 2. Moreover, additional treatments may be added. After carrying out the drawing treatment, e.g., the tube may be cleaned by degreasing it by means of liquid degreasant and also by blasting it by means of, e.g., steel or cast iron grit. Such variants are each held to be within the scope of the invention.

## Claims

1. A method of manufacturing a copper tube, which method comprises at least the following method step:
-a. the copper tube is sunk;
characterized in that the method further comprises at least the following method step:
-b. the copper tube is plastically stretched;
which method step b. is carried out after method step a.

2. A method according to claim 1, characterized in that the copper tube in method step a. is at least substantially drawn to a final dimension through sinking.

3. A method according to claim 1 or 2, characterized in that the copper tube in method step b. is plastically extended by 0.05 to 5%.

4. A method according to claim 3, characterized in that the copper tube in method step b. is extended between 0.2 and 3%.

5. A method according to any of the preceding claims, characterized in that the copper tube in step b. experiences a diameter reduction below 0.5%.

6. A method according to claim 5, characterized in that the copper tube in method step b. experiences a diameter reduction below 0.2%.

7. A method according to any of the preceding claims, characterized in that the copper tube in method step a. experiences a diameter reduction of 2-20%.

8. A method according to any of the preceding claims, characterized in that the copper tube in method step a. experiences a diameter reduction of 1-4 mm, while after carrying out method step a. the copper tube has a diameter of 6-42 mm.

9. A method according to any of the preceding claims, characterized in that method step b. is carried out immediately after method step a.

10. A method according to any of the preceding claims, characterized in that before method step a. the following method step is carried out:
-c. the copper tube is annealed for manufacturing a half-hard copper tube.

11. A method according to claim 10, characterized in that the copper tube is annealed at a temperature of 500-700°C.

12. A method according to claim 10 or 11, characterized in that before method step c. the copper tube experiences at least one drawing treatment.

13. A method according to any of the preceding claims 1-9, characterized in that before method step a. the copper tube experiences at least one drawing treatment to obtain a hard copper tube.

14. A method according to any of the preceding claims, characterized in that the starting product consists of:
1) a copper cast bar which is converted into a copper tube by means of extrusion or piercing; or
2) a cast copper tube.

15. A method according to any of the preceding claims, characterized in that after carrying out method step a. the copper tube has a residual hoop stress above 30, in particular a residual hoop stress of 30-200, and that after carrying out method step b. the copper tube has a residual hoop stress of 0-30.
